# EUROPEAN PATENT APPLICATION

(11) **EP 4 786 616 A1**
(43) Date of publication of application: **05.08.2026**
(21) Application number: 23954193.1
(22) Date of filing: 26.09.2023
(51) Int. Cl.: C22C 29/08

(54) **CEMENTED CARBIDE AND CUTTING TOOL**

(71) Applicant: Sumitomo Electric Industries, Ltd., Osaka-shi, Osaka 541-0041 (JP)
(72) Inventor: KIDO, Yasuki, Osaka-shi, Osaka 541-0041 (JP); KIMURA, Yoshihiro, Osaka-shi, Osaka 541-0041 (JP); PASEUTH, Anongsack, Osaka-shi, Osaka 541-0041 (JP); OGIWARA, Hiroyuki, Osaka-shi, Osaka 541-0041 (JP)
(74) Representative: Boult Wade Tennant LLP
(86) International application number: PCT/JP2023/035013
(87) International publication number: WO 2025/069217

(57) **Abstract**

A cemented carbide includes a plurality of tungsten carbide grains and a binder phase, wherein the cemented carbide includes the tungsten carbide grains and the binder phase in a total of 89% by volume or more, the cemented carbide includes 1.8% by volume or more and 20% by volume or less of the binder phase, the binder phase includes 80% by mass or more of cobalt, the cemented carbide includes an inner region at a distance of 300 µm or more from a surface of the cemented carbide, and in the binder phase of the inner region, a percentage { S_{(hcp)}/(S_{(hcp)} + S_{(fcc)})} × 100 of an area S_{(hcp)} of cobalt having an hcp structure to a total of the area S_{(hcp)} and an area S_{(fcc)} of cobalt having an fcc structure is 45% or more.

## Description

### TECHNICAL FIELD

The present disclosure relates to a cemented carbide and a cutting tool.

### BACKGROUND ART

Conventionally, cemented carbides comprising a plurality of tungsten carbide grains and a binder phase have been utilized as materials for cutting tools (PTL 1).

### CITATION LIST

### PATENT LITERATURE

PTL 1: Japanese Patent Laying-Open No. 2004-131769

### SUMMARY OF INVENTION

A cemented carbide according to the present disclosure is a cemented carbide comprising a plurality of tungsten carbide grains and a binder phase, wherein
the cemented carbide includes the tungsten carbide grains and the binder phase in a total of 89% by volume or more,
the cemented carbide includes 1.8% by volume or more and 20% by volume or less of the binder phase,
the binder phase includes 80% by mass or more of cobalt,
the cemented carbide includes an inner region at a distance of 300 µm or more from a surface of the cemented carbide, and
in the binder phase of the inner region, a percentage {S_{(hcp)}/(S_{(hcp)} + S_{(fcc)})} × 100 of an area S_{(hcp)} of cobalt having an hcp structure to a total of the area S_{(hcp)} and an area S_{(fcc)} of cobalt having an fcc structure is 45% or more.

### BRIEF DESCRIPTION OF DRAWINGS

[Fig. 1] Fig. 1 is a schematic cross-sectional view of a cemented carbide according to Embodiment 1.
[Fig. 2] Fig. 2 is a schematic diagram of a cutting tool according to Embodiment 2.

### DETAILED DESCRIPTION

### [Problem to be Solved by the Present Disclosure]

In recent years, workpieces have become increasingly difficult to cut in cutting processes, and the conditions under which cutting tools are used have become more severe. Therefore, a cemented carbide used as a base body of a cutting tool is also required to have improved various properties. There have been required a cemented carbide allowing for a long life of a tool particularly when the cemented carbide is used as a material of a cutting tool for intermittent processing for a high-strength material, and a cutting tool including the cemented carbide.

### [Advantageous Effect of the Present Disclosure]

According to the present disclosure, it is possible to provide a cemented carbide allowing for a long life of a tool particularly when the cemented carbide is used as a material of a cutting tool for intermittent processing for a high-strength material, and a cutting tool including the cemented carbide.

### [Description of Embodiments]

First, embodiments of the present disclosure will be listed and described.
(1) A cemented carbide according to the present disclosure is a cemented carbide comprising a plurality of tungsten carbide grains and a binder phase, wherein
   the cemented carbide includes the tungsten carbide grains and the binder phase in a total of 89% by volume or more,
   the cemented carbide includes 1.8% by volume or more and 20% by volume or less of the binder phase,
   the binder phase includes 80% by mass or more of cobalt,
   the cemented carbide includes an inner region at a distance of 300 µm or more from a surface of the cemented carbide, and
   in the binder phase of the inner region, a percentage {S_{(hcp)}/(S_{(hcp)} + S_{(fcc)})} × 100 of an area S_{(hcp)} of cobalt having an hcp structure to a total of the area S_{(hcp)} and an area S_{(fcc)} of cobalt having an fcc structure is 45% or more.
   According to the present disclosure, it is possible to provide a cemented carbide allowing for a long life of a tool particularly when the cemented carbide is used as a material of a cutting tool for intermittent processing for a high-strength material, and a cutting tool including the cemented carbide.
(2) In (1), the percentage {S_{(hcp)}/(S_{(hcp)} + S_{(fcc)})} × 100 may be 50% or more and 70% or less. According to this, deformation resistance of the binder phase is improved, with the result that a cutting tool including the cemented carbide can have a longer tool life.
(3) In (1) or (2), the binder phase may further include at least one first element selected from a group consisting of silicon, phosphorus, germanium, tin, rhenium, ruthenium, osmium, iridium, and platinum. According to this, deformation resistance of the binder phase is improved, with the result that a cutting tool including the cemented carbide can have a longer tool life.
(4) In (3), a percentage {M1/(M1 + M2)} × 100 of a mass M1 of the first element to a total M1 + M2 of the mass M1 of the first element and a mass M2 of the cobalt may be 1% or more and 6% or less. According to this, the binder phase can have both more excellent hardness and more excellent toughness, with the result that a cutting tool including the cemented carbide including the binder phase can have a longer tool life.
(5) A cutting tool of the present disclosure is a cutting tool comprising a cutting edge consisting of the cemented carbide according to any one of (1) to (4).

According to the present disclosure, it is possible to provide a cutting tool having a long tool life particularly when the cutting tool is used for intermittent processing for a high-strength material.

### [Details of Embodiments of the Present Disclosure]

Hereinafter, specific examples of the cemented carbide and cutting tool of the present disclosure will be described with reference to drawings. In the drawings of the present disclosure, the same reference signs represent the same portions or equivalent portions. In addition, dimensional relationships such as length, width, thickness, and depth are changed as appropriate for clarity and simplicity in the drawings and do not necessarily represent actual dimensional relationships.

In the present disclosure, the expression "A to B" represents a range of lower to upper limits (i.e., A or more and B or less), and in the case where no unit is indicated for A and a unit is indicated only for B, the unit of A is the same as the unit of B.

In the case where a compound or the like is expressed by a chemical formula in the present disclosure and an atomic ratio is not particularly limited, it is assumed that all the conventionally known atomic ratios are included, and the atomic ratio is not necessarily limited only to one in the stoichiometric range.

In the present disclosure, in the case where one or more numerical values are each provided as a lower limit and an upper limit of a numerical range, it is considered that a combination of any one of the numerical values provided in the lower limit and any one of the numerical values provided in the upper limit is also disclosed. For example, in the case where a1 or more, b1 or more, and c1 or more are described as lower limits, and a2 or less, b2 or less, and c2 or less are described as upper limits, it is considered that a1 or more and a2 or less, a1 or more and b2 or less, a1 or more and c2 or less, b1 or more and a2 or less, b1 or more and b2 or less, b1 or more and c2 or less, c1 or more and a2 or less, c1 or more and b2 or less, and c1 or more and c2 or less are disclosed.

### [Embodiment 1: Cemented Carbide]

A cemented carbide according to one embodiment of the present disclosure will be described with reference to Fig. 1.

A cemented carbide 3 according to one embodiment (hereinafter, also referred to as "Embodiment 1") of the present disclosure is a cemented carbide 3 comprising a plurality of tungsten carbide grains 1 and a binder phase 2, wherein
cemented carbide 3 includes tungsten carbide grains 1 and binder phase 2 in a total of 89% by volume or more,
cemented carbide 3 includes 1.8% by volume or more and 20% by volume or less of binder phase 2,
binder phase 2 includes 80% by mass or more of cobalt,
cemented carbide 3 includes an inner region at a distance of 300 µm or more from a surface of cemented carbide 3, and
in the binder phase of the inner region, a percentage {S_{(hcp)}/(S_{(hcp)} + S_{(fcc)})} × 100 of an area S_{(hcp)} of cobalt having an hcp structure to a total of the area S_{(hcp)} and an area S_{(fcc)} of cobalt having an fcc structure is 45% or more.

With the cemented carbide of Embodiment 1, it is possible to provide a cemented carbide allowing for a long life of a tool particularly when the cemented carbide is used as a material of a cutting tool for intermittent processing for a high-strength material, and a cutting tool including the cemented carbide. The reason for this is not clear, but may be presumed to be as follows.

The cemented carbide of Embodiment 1 includes the plurality of tungsten carbide grains (hereinafter, also referred to as "WC grains") and the binder phase, and a total content of the WC grains and the binder phase of the cemented carbide is 89% by volume or more. According to this, the cemented carbide has high hardness and strength, and a cutting tool including the cemented carbide can have excellent wear resistance and breakage resistance.

The cemented carbide of Embodiment 1 includes 1.8% by volume or more and 20% by volume or less of the binder phase, and the binder phase includes 80% by mass or more of the cobalt. According to this, the cemented carbide has high hardness and strength, and a cutting tool including the cemented carbide can have excellent wear resistance and breakage resistance.

In the binder phase of the inner region of the cemented carbide of Embodiment 1, the percentage {S_{(hcp)}/(S_{(hcp)} + S_{(fcc)})} × 100 of the area S_{(hcp)} of the cobalt having the hcp structure to the total of the area S_{(hcp)} and the area S_{(fcc)} of the cobalt having the fcc structure is 45% or more. According to this, deformation resistance of the binder phase is improved, thereby improving deformation resistance of the cemented carbide.

### <Composition of Cemented Carbide>

The cemented carbide of Embodiment 1 includes the tungsten carbide grains and the binder phase in a total of 89% by volume or more. As a result, the hardness of the cemented carbide can be enhanced. The cemented carbide may include the tungsten carbide grains and the binder phase in a total of 89% by volume or more and 100% by volume or less, may include them in a total of 90% by volume or more and 100% by volume or less, may include them in a total of 91% by volume or more and 100% by volume or less, or may include them in a total of 92% by volume or more and 100% by volume or less.

The cemented carbide of Embodiment 1 includes 1.8% by volume or more and 20% by volume or less of the binder phase. As a result, the hardness and toughness of the cemented carbide can be enhanced. The content of the binder phase in the cemented carbide may be 2.0% by volume or more and 19.0% by volume or less, may be 3.0% by volume or more and 18.0% by volume or less, or may be 4.0% by volume or more and 17.0% by volume or less.

The cemented carbide of Embodiment 1 can consist of the plurality of tungsten carbide grains and the binder phase. In this case, the cemented carbide can include impurities to the extent that the effects of the present disclosure are not impaired.

In addition to the tungsten carbide grains and the binder phase, the cemented carbide can include other phases (not shown). Examples of the other phases include carbides, nitrides, or carbonitrides including at least one element selected from the group consisting of titanium (Ti), tantalum (Ta), niobium (Nb), zirconium (Zr), hafnium (Hf), and molybdenum (Mo). The composition of the other phases may be, for example, at least one selected from the group consisting of TiCN, TaC, NbC, ZrC, HfC, Cr₃C₂, and Mo₂C.

The cemented carbide of Embodiment 1 can consist of the tungsten carbide grains, the binder phase, and the other phases. In this case, the cemented carbide can include impurities to the extent that the effects of the present disclosure are not impaired.

The content of the other phases in the cemented carbide is permissible to the extent that the effects of the present disclosure are not impaired. For example, the content of the other phases in the cemented carbide may be 0% by volume or more and 11% by volume or less, may be more than 0% by volume and 11% by volume or less, may be more than 0% by volume and 7% by volume or less, or may be more than 0% by volume and 4% by volume or less.

The cemented carbide of Embodiment 1 can include impurities. Examples of the impurities include iron (Fe), calcium (Ca), silicon (Si), and sulfur (S). The content of the impurities in the cemented carbide is permissible to the extent that the effects of the present disclosure are not impaired. For example, the content of the impurities in the cemented carbide may be 0% by mass or more and less than 0.1% by mass. The content of the impurities in the cemented carbide is measured by inductively coupled plasma (ICP) emission spectroscopy. "ICPS-8100" (TM) manufactured by Shimadzu Corporation can be used as the measurement device.

The content of the tungsten carbide grains in the cemented carbide of Embodiment 1 may be 67% by volume or more and 98.2% by volume or less, may be 70% by volume or more and 97% by volume or less, or may be 75% by volume or more and 96% by volume or less.

The method for measuring the content of the tungsten carbide grains in the cemented carbide (% by volume) and the content of the binder phase in the cemented carbide (% by volume) is as follows.

(A1) The cemented carbide is cut out at any position to expose a cross-section. The cross-section is subjected to mirror surface processing using CROSS SECTION POLISHER (manufactured by JEOL Ltd.).

(B1) The surface of the cemented carbide that has been subjected to the mirror surface processing is analyzed using an energy dispersive X-ray spectrometer attached to a scanning electron microscope (SEM-EDX) (device: "Gemini 450" (TM) manufactured by Carl Zeiss AG) to identify the elements included in the cemented carbide.

(C1) The surface of the cemented carbide that has been subjected to the mirror surface processing is imaged using a scanning electron microscope (SEM) to obtain a backscattered electron image. The region to be imaged is set at the center of the cross-section of the cemented carbide, i.e., at a position that does not include portions where the properties clearly differ from those of the bulk portion, such as the vicinity of the surface of the cemented carbide (at a position where the entire region to be imaged is the bulk portion of the cemented carbide). The observation magnification is 5000 times. The measurement conditions are an acceleration voltage of 3 kV, a current value of 2 nA, and a working distance (WD) of 5 mm.

(D1) The region to be imaged in the above (C1) is analyzed using SEM-EDX to identify the distribution of the elements identified in the above (B1) in the region to be imaged, and an elemental mapping image is obtained.

(E1) The backscattered electron image obtained in the above (C1) is imported into a computer and subjected to a binarization process using image analysis software (OpenCV, SciPy). In the image after the binarization process, the tungsten carbide grains are shown in white, and the binder phase is shown in gray to black. Note that the threshold value of the binarization varies depending on the contrast, and is thus set for each image.

(F1) The elemental mapping image obtained in the above (D1) and the image after the binarization process obtained in the above (E1) are overlapped, thereby identifying the respective regions where the tungsten carbide grains and the binder phase are present on the image after the binarization process. Specifically, the region shown in white in the image after the binarization process and the region where tungsten (W) and carbon (C) are present in the elemental mapping image correspond to the region where the tungsten carbide grains are present. The region shown in gray to black in the image after the binarization process and the region where cobalt (Co) is present in the elemental mapping image correspond to the region where the binder phase is present.

(G1) In the image after the binarization process, a rectangular measurement field of 24.9 µm × 18.8 µm is set. Using the above image analysis software, the respective area percentages of the tungsten carbide grains and the binder phase are measured with the area of the entire measurement field as the denominator.

(H1) The measurement of the above (G1) is performed at five different measurement fields that are not overlapped with each other. In the present disclosure, the average of the area percentages of the tungsten carbide grains in the five measurement fields corresponds to the content (% by volume) of the tungsten carbide grains in the cemented carbide, and the average of the area percentages of the binder phase in the five measurement fields corresponds to the content (% by volume) of the binder phase in the cemented carbide.

In the case where the cemented carbide includes other phases in addition to the WC grains and the binder phase, the content of the other phases in the cemented carbide can be obtained by subtracting the content (% by volume) of the tungsten carbide grains and the content (% by volume) of the binder phase as measured in the above procedure from the entire cemented carbide (100% by volume).

It has been confirmed that, as long as measurement is performed on the same sample, even if the cut-out location for the cross-section of the cemented carbide, the region to be imaged described in the above (C1), and the measurement field described in the above (G1) are arbitrarily set and the measurement of the content of the tungsten carbide grains and the content of the binder phase in the cemented carbide is performed multiple times according to the above procedure, there is little variation in the measurement results.

The cemented carbide of Embodiment 1 may include 1% by mass or more of cobalt. The cobalt content in the cemented carbide may be 1.0% by mass or more and 20% by mass or less, may be 2.0% by mass or more and 15% by mass or less, or may be 3.0% by mass or more and 12% by mass or less.

A method for measuring the content of cobalt in the cemented carbide is as follows. By the same method as (A1) to (D1) of the method for measuring the content of the tungsten carbide grains and the content of the binder phase in the cemented carbide described above, analysis using SEM-EDX is performed to obtain an elemental mapping image. Based on the elemental mapping image, the region of cobalt in the cemented carbide is identified and the content of cobalt is measured. The measurement is performed at five different regions to be imaged that are not overlapped with each other. In the present disclosure, the average of the contents of cobalt in the five regions to be imaged corresponds to the content of cobalt in the cemented carbide.

It has been confirmed that, as long as measurement is performed on the same sample, even if the cut-out location for the cross-section of the cemented carbide and the region to be imaged described in the above (C1) are arbitrarily set and the measurement of the content of cobalt in the cemented carbide is performed multiple times according to the above procedure, there is little variation in the measurement results.

### <Tungsten Carbide Grains>

In the cemented carbide of Embodiment 1, the tungsten carbide grains include at least any of "pure WC grains (including WC not containing any impurity elements, as well as WC in which the content of impurity elements is below the detection limit)" and "WC grains in which impurity elements are intentionally or inevitably contained therein to the extent that the effects of the present disclosure are not impaired". The content of impurities in the tungsten carbide grains (in the case where there are two or more elements constituting the impurities, their total concentration) is less than 0.1% by mass. The content of impurity elements in the tungsten carbide grains is measured by ICP emission spectroscopy.

In Embodiment 1, the average grain size of the tungsten carbide grains is not particularly restricted. The average grain size of the tungsten carbide grains can be, for example, 0.1 µm or more and 3.5 µm or less. It has been confirmed that the cemented carbide of Embodiment 1 enables a longer life of tools in the case where it is used as a material for cutting tools, regardless of the average grain size of the tungsten carbide grains.

### <Binder Phase>

In the cemented carbide of Embodiment 1, the binder phase includes 80% by mass or more of cobalt. As a result, the cemented carbide can have excellent toughness. The cobalt content in the binder phase may be 80% by mass or more and 100% by mass or less, may be 80% by mass or more and less than 100% by mass, or may be 90% by mass or more and less than 100% by mass.

A method for measuring the content of cobalt in the binder phase is as follows. By the same method as (A1) to (E1) of the method for measuring the content of the tungsten carbide grains and the content of the binder phase in the cemented carbide described above, an elemental mapping image and an image after the binarization process are obtained. The elemental mapping image and the image after the binarization process are overlapped, thereby identifying the region where the binder phase is present on the elemental mapping image. In the elemental mapping image, one rectangular measurement field of 24.9 µm × 18.8 µm is set. In the region where the binder phase is present in the measurement field, the cobalt content is measured. The above measurement is performed at five different measurement fields that are not overlapped with each other. In the present disclosure, the average of the cobalt contents in the region where the binder phase is present in the five measurement fields corresponds to the cobalt content in the binder phase.

It has been confirmed that, as long as measurement is performed on the same sample, even if the cut-out location for the cross-section of the cemented carbide, the region to be imaged described in the above (C1), and the above measurement field are arbitrarily set and the measurement of the cobalt content in the binder phase is performed multiple times according to the above procedure, there is little variation in the measurement results.

In the cemented carbide of Embodiment 1, the binder phase may further include at least one first element selected from the group consisting of silicon, phosphorus, germanium, tin, rhenium, ruthenium, osmium, iridium, and platinum. Thus, deformation resistance of the binder phase is improved.

Whether the binder phase includes the first element is confirmed by the following procedure. By the same method as (A1) to (E1) of the method for measuring the content of the tungsten carbide grains and the content of the binder phase in the cemented carbide described above, an elemental mapping image and an image after the binarization process are obtained. The elemental mapping image and the image after the binarization process are overlapped, thereby identifying the region where the binder phase is present on the elemental mapping image. In the elemental mapping, in the case where the first element is present in the region where the binder phase is present, it is confirmed that the binder phase includes the first element.

In the binder phase of the cemented carbide of Embodiment 1, the percentage {M1/(M1 + M2)} × 100 of the mass M1 of the first element to the total M1 + M2 of the mass M1 of the first element and the mass M2 of cobalt may be 1% or more and 6% or less. Here, the units of M1 and M2 are the same. As a result, the binder phase can have more excellent hardness and more excellent toughness in combination, and therefore, a cutting tool comprising a cemented carbide comprising the binder phase can have a longer tool life. Here, the mass M1 of the first element means, in the case where the binder phase includes two or more first elements, the total mass of all first elements. The percentage {M1/(M1 + M2)} × 100 may be 2% or more and 5% or less, or may be 3% or more and 4% or less.

A method for measuring the above percentage {M1/(M1 + M2)} × 100 is as follows. By the same method as (A1) to (E1) of the method for measuring the content of the tungsten carbide grains and the content of the binder phase in the cemented carbide described above, an elemental mapping image and an image after the binarization process are obtained. The elemental mapping image and the image after the binarization process are overlapped, thereby identifying the region where the binder phase is present on the elemental mapping image. In the elemental mapping image, one rectangular measurement field of 24.9 µm × 18.8 µm is set. In the region where the binder phase is present in the measurement field, the percentage {m1/(m1 + m2)} × 100 of the mass m1 of the first element to the total m1 + m2 of the mass m1 of the first element and the mass m2 of cobalt is calculated. The above measurement is performed at five different measurement fields that are not overlapped with each other. In the present disclosure, the average of the percentages {m1/(m1 + m2)} × 100 in the five measurement fields corresponds to "the percentage {M1/(M1 + M2)} × 100" in the binder phase of the cemented carbide.

It has been confirmed that, as long as measurement is performed on the same sample, even if the cut-out location for the cross-section of the cemented carbide, the region to be imaged described in the above (C 1), and the above measurement field are arbitrarily set and the measurement of the percentage {M1/(M1 + M2)} × 100 is performed multiple times according to the above procedure, there is little variation in the measurement results.

In the cemented carbide of Embodiment 1, the binder phase can include at least one second element selected from the group consisting of iron, nickel, and chromium in addition to cobalt and the first element. The binder phase can consist of cobalt, the first element, and the second element. The binder phase can consist of cobalt, the first element, the second element, and inevitable impurities. Examples of the inevitable impurities include iron, nickel, and sulfur.

### <Percentage { S_{(hcp)}/(S_{(hcp)} + S_{(fcc)})} × 100 of Binder Phase of Inner Region>

The cemented carbide of the Embodiment 1 includes the inner region at the distance of 300 µm or more from the surface of the cemented carbide, and in the binder phase of the inner region, the percentage { S_{(hcp)}/(S_{(hcp)} + S_{(fcc)})} × 100 of the area S_{(hcp)} of the cobalt having the hcp (hexagonal close-packed) structure to the total of the area S_{(hcp)} and the area S_{(fcc)} of the cobalt having the fcc (face-centered cubic) structure is 45% or more. The percentage { S_{(hcp)}/(S_{(hcp)} + S_{(fcc)})} × 100 may be 45% or more and 80% or less, or 50% or more and 70% or less.

In the present disclosure, the percentage { S_{(hcp)}/(S_{(hcp)} + S_{(fcc)})} × 100 in the binder phase of the inner region of the cemented carbide is measured by the following procedure.

(A2) The cemented carbide is cut along a normal line of its main surface to expose a cross-section. When the surface of the cemented carbide does not have a flat region, the cemented carbide is cut out from any point on the surface along a direction toward the center of gravity of the cemented carbide so as to expose a cross-section. The cross-section is subjected to mirror surface processing using CROSS SECTION POLISHER (manufactured by JEOL Ltd.).

(B2) The surface of the cemented carbide that has been subjected to the mirror surface processing is observed using a scanning electron microscope (SEM device: "Gemini 450" (TM) manufactured by Carl Zeiss AG) including an electron backscatter diffraction pattern device (EBSD device: "Symmetry" (TM) manufactured by Oxford Instruments). The obtained observation image is subjected to an EBSD analysis. The observation image is acquired to include the inner region at the distance of 300 µm or more from the surface of the cemented carbide. A rectangular measurement field of 11.5 µm × 8.5 µm is set in the inner region of the observation image. The observation magnification is 10,000 times. The measurement conditions are an acceleration voltage of 15 kV, a current value of 20 nA, 0.02 µm/step, an exposure time of 1.5 to 3 ms, and a measurement time of 10 to 20 minutes hours.

(C2) The result of the EBSD analysis is analyzed using commercially available software ("AZtecCrystal" (TM) manufactured by Oxford Instruments) to identify the crystal structure of the cobalt included in the binder phase in the measurement field, thereby obtaining a color map. The crystal structure of the cobalt identified herein is a crystal structure observed when the cobalt that appears in the surface of the cemented carbide that has been subjected to the mirror surface processing is viewed in plan in a normal direction of the surface that has been subjected to the mirror surface processing.

(D2) The above software is used to measure the percentage {S_{(hcp)}/(S_{(hcp)} + S_{(fcc)})} × 100 of the area S_{(hcp)} of the cobalt having the hcp structure to the total of the area S_{(hcp)} and the area S_{(fcc)} of the cobalt having the fcc structure in the binder phase of the measurement field. For example, an image A, in which the tungsten carbide grains are shown in white and the cobalt having the hcp structure is shown in black, and an image B, in which the tungsten carbide grains are shown in white and the cobalt having the fcc structure is shown in black, are output based on the color map, and the percentage {S_{(hcp)}/(S_{(hcp)} + S_{(fcc)})} × 100 can be measured based on the image A and the image B.

(E2) The above measurement of the percentage {S_{(hcp)}/(S_{(hcp)} + S_{(fcc)})} × 100 is performed in three different measurement fields that are not overlapped with each other. In the present disclosure, the average of the percentages { S_{(hcp)}/(S_{(hcp)} + S_{(fcc)})} × 100 in the three measurement fields corresponds to the percentage { S_{(hcp)}/(S_{(hcp)} + S_{(fcc)})} × 100 in the binder phase of the inner region of the cemented carbide.

It has been confirmed that, as long as measurement is performed on the same sample, even if the cut-out location for the cross-section of the cemented carbide, the region for which the observation image described in (B2) above is to be acquired, and the measurement field are arbitrarily set and the measurement of the percentage {S(_{hcp})/(S_{(hcp)} + S_{(fcc)})} × 100 in the binder phase of the inner region of the cemented carbide is performed multiple times according to the above procedure, there is little variation in the measurement results.

The cemented carbide of Embodiment 1 may include a surface region at a distance of less than 300 µm from the surface of the cemented carbide. The percentage { S_{(hcp)}/(S_{(hcp)} + S_{(fcc)})} × 100 in the binder phase of the surface region of the cemented carbide of Embodiment 1 is not particularly limited. This is due to the following reason: when forming, by grinding, the cutting edge of the cutting tool consisting of the cemented carbide, the surface region of the cemented carbide is affected by stress during the grinding and is therefore not an essential portion of the cemented carbide that directly affects the life of the cutting tool. On the other hand, the inner region at the distance of 300 µm or more from the surface of the cemented carbide is the essential portion of the cemented carbide that affects the life of the cutting tool because the inner region is less likely to receive stress when forming the cutting edge of the cutting tool by the grinding. Thus, in the cemented carbide of the present disclosure, the percentage { S_{(hcp)}/(S_{(hcp)} + S_{(fcc)})} × 100 in the binder phase of the inner region is defined. The percentage { S_{(hcp)}/(S_{(hcp)} + S_{(fcc)})} × 100 in the binder phase of the surface region of the cemented carbide of Embodiment 1 may be, for example, less than 45%.

### <Method for Producing Cemented Carbide>

The cemented carbide of Embodiment 1 can be produced by performing a raw material powder preparation step, a mixing step, a molding step, and a sintering step in this order. Each step will be described below.

### <Preparation Step>

The preparation step is a step of preparing raw material powders of the cemented carbide. Examples of the raw material powders include a tungsten carbide powder (hereinafter, also referred to as "WC powder"), a cobalt (Co) powder, a first element powder, and an alloy powder of the first element and cobalt. Examples of the first element powder include a silicon (Si) powder, a phosphorus (P) powder, a germanium (Ge) powder, a tin (Sn) powder, a rhenium (Re) powder, a ruthenium (Ru) powder, an osmium (Os) powder, an iridium (Ir) powder, and a platinum (Pt) powder. As the raw material powders, a nickel (Ni) powder, a niobium carbide (NbC) powder, a tungsten carbide (TaC) powder, a titanium carbonitride (TiCN) powder, a chromium carbide (Cr₃C₂) powder, and other powders can be further prepared. As these raw material powders, those commercially available can be used. The average grain size of these raw material powders is not particularly restricted, and it can be 0.5 to 2 µm, for example. The average grain size of the raw material powders means an average grain size measured by the Fisher Sub-Sieve Sizer (FSSS) method. The average grain size is measured using "Sub-Sieve Sizer Model 95" (TM) manufactured by Fisher Scientific International, Inc.

### <Mixing Step>

The mixing step is a step of mixing each raw material powder prepared in the preparation step at a predetermined proportion. A mixed powder in which each raw material powder is mixed is obtained by the mixing step. The mixing proportion of each raw material powder is adjusted as appropriate depending on the composition of the target cemented carbide.

For the mixing of each raw material powder, conventionally known mixing methods such as attritors, ball mills, and bead mills can be used. The mixing conditions used can also be conventionally known conditions. The mixing time can be 2 hours or longer and 20 hours or shorter, for example.

After the mixing step, the mixed powder may be granulated as necessary. By granulating the mixed powder, it is easy to fill the mixed powder into a die or mold during the molding step described later. Known granulation methods can be applied for the granulation, and for example, a commercially available granulator such as a spray dryer can be used.

### <Molding Step>

The molding step is a step of molding the mixed powder obtained in the mixing step into a shape for cutting tools to obtain a molded body. The molding method and molding conditions in the molding step are not particularly restricted as long as general methods and conditions may be employed.

### <Sintering Step>

The sintering step is a step of sintering the molded body obtained in the molding step to obtain a cemented carbide intermediate. Specifically, the molded body is held under conditions of 7 MPa and 1360°C for 2 hours.

### <Cooling Step>

The cooling step is a step of cooling the cemented carbide intermediate after the sintering step. Specifically, the cemented carbide intermediate is cooled to 1200°C in vacuum and is held for 30 minutes. Then, the cemented carbide intermediate is gradually cooled in vacuum to 1000°C at a temperature decrease rate of -0.5°C/min. Then, the cemented carbide intermediate is rapidly cooled in vacuum to the room temperature (23°C) at a temperature decrease rate of -20°C/min, thereby obtaining the cemented carbide of Embodiment 1.

### <Features of Method for Producing Cemented Carbide of Embodiment 1>

In the method for producing a cemented carbide according to Embodiment 1, the sintering step is performed by holding the cemented carbide intermediate under conditions of 7 MPa and 1360°C for 2 hours. Moreover, in the cooling step, the cemented carbide intermediate is cooled to 1200°C in vacuum and is held for 30 minutes, is then gradually cooled to 1000°C in vacuum at the temperature decrease rate of -0.5°C/min, and is then rapidly cooled to the room temperature (23°C) in vacuum at the temperature decrease rate of -20°C/min. With these conditions, it is possible to produce the cemented carbide of Embodiment 1 in which the percentage { S_{(hcp)}/(S_{(hcp)} + S_{(fcc)})} × 100 in the binder phase of the inner region of the cemented carbide is 45% or more. As a result of diligent study, the present inventors have found that the cemented carbide of the present disclosure can be realized by employing such a sintering step and such a cooling step.

### [Embodiment 2: Cutting Tool]

A cutting tool of one embodiment of the present disclosure (hereinafter, also referred to as "Embodiment 2") includes a cutting edge consisting of the cemented carbide of Embodiment 1. In the present disclosure, the cutting edge means the portion involved in cutting. More specifically, the cutting edge means the region bounded by the cutting edge ridgeline and a hypothetical plane at a distance of 0.5 mm or 2 mm from the cutting edge ridgeline to the cemented carbide side.

As the cutting tool, for example, cutting bits, drills, end mills, indexable cutting inserts for milling, indexable cutting inserts for turning, metal saws, gear cutting tools, reamers, or taps, etc. can be exemplified. As shown in Fig. 2, a cutting tool 10 of Embodiment 2 can exhibit excellent effects particularly in the case where it is an end mill. A cutting edge 11 of cutting tool 10 shown in Fig. 2 consists of the cemented carbide of Embodiment 1.

In the cutting tool of Embodiment 2, the cemented carbide of Embodiment 1 may constitute the entirety of this tool, or may constitute part of it. Here, "constitute part of it" indicates an aspect in which the cemented carbide of Embodiment 1 is brazed to a predetermined position of any base body to make a cutting edge portion, etc.

The cutting tool of Embodiment 2 may further include a hard film covering at least part of the surface of a base body consisting of the cemented carbide. As the hard film, for example, diamond-like carbon or diamond can be used.

The cutting tool of Embodiment 2 can be obtained by molding the cemented carbide of Embodiment 1 into the desired shape.

### EXAMPLES

The present embodiment will be described more specifically with reference to examples. However, the present embodiment is not limited by these examples.

### [Production of Cemented Carbide]

A cemented carbide of each sample was produced by the following procedure.

### <Preparation Step>

As raw material powders, a WC powder (average grain size: 1 µm), a Co powder (average grain size: 1 µm), a first element powder, a TiCN powder (average grain size: 1 µm), a Cr₃C₂ powder (average grain size: 1 µm), and a Ni powder (average grain size: 1 µm) were prepared. As the first element powder, a silicon (Si) powder (average grain size: 1 µm), a phosphorus (P) powder (average grain size: 1 µm), a germanium (Ge) powder (average grain size: 1 µm), a tin (Sn) powder (average grain size: 1 µm), a rhenium (Re) powder (average grain size: 1 µm), a ruthenium (Ru) powder (average grain size: 1 µm), an osmium (Os) powder (average grain size: 1 µm), an iridium (Ir) powder (average grain size: 1 µm), and a platinum (Pt) powder (average grain size: 1 µm) were prepared.

### <Mixing Step>

Each raw material powder was mixed in the proportion described in Table 1 for 10 hours using an attritor to obtain a mixed powder. The proportion (% by mass) of each raw material powder described in Table 1 is the proportion in the case where the entire mixed powder is 100% by mass.

### [Table 1]

**Table 1**

| Sample No. | Mixing step | | | | | |
|---|---|---|---|---|---|---|
| | WC powder | Co powder | First element powder | | Other powder | |
| | % by mass | % by mass | Type | % by mass | Type | % by mass |
| 1 | 91.7 | 8.0 | Si | 0.3 | - | - |
| 2 | 91.9 | 8.0 | P | 0.1 | - | - |
| 3 | 91.8 | 8.0 | Ge | 0.2 | - | - |
| 4 | 91.75 | 8.0 | Sn | 0.25 | - | - |
| 5 | 91.6 | 8.0 | Re | 0.4 | - | - |
| 6 | 98.96 | 1.0 | Re | 0.04 | - | - |
| 7 | 87.1 | 12.5 | Re | 0.4 | - | - |
| 8 | 87.6 | 8.0 | Re | 0.4 | TiCN | 4 |
| 9 | 90.8 | 8.0 | Re | 0.4 | Cr₃C₂ | 0.8 |
| 10 | 92.0 | 6.4 | Re | 0.4 | Ni | 1.2 |
| 11 | 91.9 | 8.0 | Re | 0.1 | - | - |
| 12 | 91.6 | 8.0 | Re, Si | Re: 0.2 | - | - |
| | | | | Si: 0.2 | | |
| 13 | 91.45 | 8.0 | Ru | 0.55 | - | - |
| 14 | 91.7 | 8.0 | Os | 0.3 | - | - |
| 15 | 91.8 | 8.0 | Ir | 0.2 | - | - |
| 16 | 91.75 | 8.0 | Pt | 0.25 | - | - |
| 101 | 99.17 | 0.8 | Re | 0.03 | - | - |
| 102 | 86.5 | 13.0 | Re | 0.5 | - | - |
| 103 | 87.1 | 8.0 | Re | 0.4 | TiCN | 4.5 |
| 104 | 92.1 | 6.2 | Re | 0.3 | Ni | 1.4 |
| 105 | 92.0 | 8.0 | - | - | - | - |
| 106 | 91.95 | 8.0 | Re | 0.05 | - | - |
| 107 | 91.6 | 8.0 | Re | 0.4 | - | - |

### <Molding Step>

The mixed powder was pressed to obtain a round bar-shaped molded body.

### <Sintering Step>

The molded body was held at the pressure described in the "Holding pressure" column and the temperature described in the "Holding temperature" column of the "sintering step" in Table 2 for the time described in the "Holding time" column. As a result, a cemented carbide intermediate was obtained.

### <Cooling Step>

For each of Samples 1 to 16 and Samples 101 to 105, the cemented carbide intermediate after the sintering step was cooled in the following procedure to obtain the cemented carbide. The cemented carbide intermediate was cooled in vacuum to 1200°C (described in the "First cooling temperature" column of Table 2) and was held for 30 minutes (described in the "First holding time" column of Table 2). Then, the cemented carbide intermediate was gradually cooled in vacuum to 1000°C at a temperature decrease rate of -0.5°C/min (described in the "Temperature decrease rate to 1000°C" column in Table 2). Then, the cemented carbide intermediate was rapidly cooled in vacuum to the room temperature (23°C) at a temperature decrease rate of - 20°C/min (described in the "Temperature decrease rate to 23°C" column of Table 2), thereby obtaining the cemented carbide of each sample.

In each of Samples 106 and 107, the cemented carbide intermediate after the sintering step was rapidly cooled in vacuum to the room temperature (23°C) at a temperature decrease rate of -20°C/min (described in the "Temperature decrease rate to 23°C" column of Table 2), thereby obtaining the cemented carbide of each sample.

### [Table 2]

**Table 2**

| Sample No. | Sintering step | | | Cooling step | | | |
|---|---|---|---|---|---|---|---|
| | Holding temperature | Holding pressure | Holding time | First cooling temperature | First holding time | Temperature decrease rate to 1000°C | Temperature decrease rate to 23°C |
| | °C | MPa | hr | °C | min | °C/min | °C/min |
| 1 | 1360 | 7 | 2 | 1200 | 30 | -0.5 | -20 |
| 2 | 1360 | 7 | 2 | 1200 | 30 | -0.5 | -20 |
| 3 | 1360 | 7 | 2 | 1200 | 30 | -0.5 | -20 |
| 4 | 1360 | 7 | 2 | 1200 | 30 | -0.5 | -20 |
| 5 | 1360 | 7 | 2 | 1200 | 30 | -0.5 | -20 |
| 6 | 1360 | 7 | 2 | 1200 | 30 | -0.5 | -20 |
| 7 | 1360 | 7 | 2 | 1200 | 30 | -0.5 | -20 |
| 8 | 1360 | 7 | 2 | 1200 | 30 | -0.5 | -20 |
| 9 | 1360 | 7 | 2 | 1200 | 30 | -0.5 | -20 |
| 10 | 1360 | 7 | 2 | 1200 | 30 | -0.5 | -20 |
| 11 | 1360 | 7 | 2 | 1200 | 30 | -0.5 | -20 |
| 12 | 1360 | 7 | 2 | 1200 | 30 | -0.5 | -20 |
| 13 | 1360 | 7 | 2 | 1200 | 30 | -0.5 | -20 |
| 14 | 1360 | 7 | 2 | 1200 | 30 | -0.5 | -20 |
| 15 | 1360 | 7 | 2 | 1200 | 30 | -0.5 | -20 |
| 16 | 1360 | 7 | 2 | 1200 | 30 | -0.5 | -20 |
| 101 | 1360 | 7 | 2 | 1200 | 30 | -0.5 | -20 |
| 102 | 1360 | 7 | 2 | 1200 | 30 | -0.5 | -20 |
| 103 | 1360 | 7 | 2 | 1200 | 30 | -0.5 | -20 |
| 104 | 1360 | 7 | 2 | 1200 | 30 | -0.5 | -20 |
| 105 | 1360 | 7 | 2 | 1200 | 30 | -0.5 | -20 |
| 106 | 1360 | 0.1 kPa | 1 | - | - | - | -20 |
| 107 | 1360 | 0.1 kPa | 1 | - | - | - | -20 |

### [Evaluation of Cemented Carbide]

### <Content (% by volume) of Tungsten Carbide Grains and Content (% by volume) of Binder Phase in Cemented Carbide>

The content (% by volume) of the tungsten carbide grains and the content (% by volume) of the binder phase in the cemented carbide of each sample were measured. A specific measurement method is as described in Embodiment 1. The results are shown in the "WC grain content" and "Binder phase content" columns of "Cemented carbide" in Table 3. Furthermore, the total of the content of the tungsten carbide grains and the content of the binder phase in the cemented carbide is shown in the "WC grain + binder phase content" column of "Cemented carbide" in Table 3. **In** Table 3, cemented carbides in which the "WC grain + binder phase content" column is less than 100% by volume were confirmed to further include TiCN or Cr₃C₂.

### [Table 3]

**Table 3**

| Sample No. | Cemented carbide | | |
|---|---|---|---|
| | WC grain content | Binder phase content | WC grain + binder phase content |
| | % by volume | % by volume | % by volume |
| 1 | 85.2 | 14.8 | 100 |
| 2 | 86.1 | 13.9 | 100 |
| 3 | 86.3 | 13.7 | 100 |
| 4 | 86.4 | 13.6 | 100 |
| 5 | 86.5 | 13.5 | 100 |
| 6 | 98.2 | 1.8 | 100 |
| 7 | 80.0 | 20.0 | 100 |
| 8 | 76.5 | 12.5 | 89 |
| 9 | 84.7 | 13.3 | 98 |
| 10 | 88.9 | 11.1 | 100 |
| 11 | 86.9 | 13.1 | 100 |
| 12 | 86.8 | 13.2 | 100 |
| 13 | 86.2 | 13.8 | 100 |
| 14 | 86.8 | 13.2 | 100 |
| 15 | 86.8 | 13.2 | 100 |
| 16 | 86.7 | 13.3 | 100 |
| 101 | 98.5 | 1.5 | 100 |
| 102 | 79.5 | 20.5 | 100 |
| 103 | 74.7 | 12.3 | 87 |
| 104 | 89.4 | 10.6 | 100 |
| 105 | 87.0 | 13.0 | 100 |
| 106 | 86.9 | 13.1 | 100 |
| 107 | 86.5 | 13.3 | 100 |

### <Cobalt Content in Binder Phase>

In the cemented carbide of each sample, the cobalt content in the binder phase was measured. A specific measurement method is as described in Embodiment 1. The results are shown in the "Co content" column of "Binder phase" in Table 4.

### <Type of First Element and {M1/(M1 + M2)} × 100>

In the binder phase of the cemented carbide of each sample, the type of the first element and the percentage {M1/(M1 + M2)} × 100 of the mass M1 of the first element to the total M1 + M2 of the mass M1 of the first element and the mass M2 of cobalt were measured. A specific measurement method is as described in Embodiment 1. The results are shown in the "First element" column and the "{M1/(M1 + M2)} × 100" column of "Binder phase" in Table 4. Samples with "-" noted in the "First element" column indicate that they do not include the first element.

### <{S_{(hcp)}/(S_{(hcp)} + 3_{(fcc)})} × 100>

In the binder phase of the inner region of each sample at the distance of 300 µm or more from the surface of the cemented carbide, the percentage { S_{(hcp)}/(S_{(hcp)} + S_{(fcc)})} × 100 of the area S_{(hcp)} of the cobalt having the hcp structure to the total of the area S_{(hcp)} and the area S_{(fcc)} of the cobalt having the fcc structure was measured. A specific measurement method is as described in Embodiment 1. The results are shown in the "{S_{(hcp)}/(S_{(hcp)} + S_{(fcc)})} × 100" column of the "Binder phase" in Table 4.

### [Cutting Test]

The round bar consisting of the cemented carbide of each sample was processed to produce a radius end mill having a cutting edge diameter φ of 6 mm. The radius end mill was used to perform side-surface intermittent processing onto an Inconel 718 aged material (holes with φ of 2 mm are provided at equal intervals). The processing conditions were as follows: a cutting speed Vc of 30 m/min, one cutting edge feed fz of 0.1 mm/cutting edge, a cut-in amount (axial direction) ap of 3.0 mm, a cut-in amount (radial direction) ae of 1.0 mm, and wet processing. A cutting length until occurrence of chipping of the cutting edge was measured. It is indicated that as the cutting length is longer, the tool life is longer. The results are shown in the "Cutting length" column of the "Cutting test" in Table 4. Note that the above processing conditions correspond to the intermittent processing for a high-strength material.

### [Table 4]

**Table 4**

| Sample No. | Binder phase | | | | Cutting test |
|---|---|---|---|---|---|
| | Co content | First element | {M1/(M1+M2)} x100 | {S_{(hcp)}/(S_{(hcp)}+S_{(fcc)})} ×100 | Cutting length |
| | % by mass | Type | % | % | m |
| 1 | 96 | Si | 3.7 | 58 | 10.2 |
| 2 | 99 | P | 1.2 | 59 | 10.2 |
| 3 | 98 | Ge | 2.3 | 68 | 10.8 |
| 4 | 97 | Sn | 2.9 | 65 | 10.5 |
| 5 | 95 | Re | 4.7 | 63 | 10.5 |
| 6 | 96 | Re | 3.7 | 60 | 10.2 |
| 7 | 97 | Re | 3.0 | 70 | 11.1 |
| 8 | 95 | Re | 4.7 | 63 | 10.5 |
| 9 | 95 | Re | 4.8 | 55 | 9.9 |
| 10 | 80 | Re | 5.9 | 54 | 9.9 |
| 11 | 99 | Re | 1.1 | 45 | 9.3 |
| 12 | 95 | Re,Si | 5.0 | 57 | 10.2 |
| 13 | 94 | Ru | 6.2 | 53 | 9.3 |
| 14 | 97 | Os | 3.5 | 55 | 9.9 |
| 15 | 98 | Ir | 2.5 | 58 | 10.2 |
| 16 | 97 | Pt | 3.0 | 57 | 9.9 |
| 101 | 97 | Re | 3.5 | 47 | 5.7 |
| 102 | 96 | Re | 3.6 | 48 | 6.3 |
| 103 | 95 | Re | 4.7 | 50 | 6.3 |
| 104 | 78 | Re | 4.7 | 52 | 6.6 |
| 105 | 100 | - | 0 | 43 | 6.0 |
| 106 | 99 | Re | 0.6 | 38 | 5.1 |
| 107 | 95.2 | Re | 4.4 | 41 | 5.7 |

### [Discussion]

The cemented carbides and cutting tools of Sample 1 to Sample 16 correspond to Examples. The cemented carbides and cutting tools of Sample 101 to Sample 107 correspond to Comparative Examples. It was confirmed that the cutting tools of Sample 1 to Sample 16 had a longer tool life than those of the cutting tools of Sample 101 to Sample 107.

Heretofore, the embodiments and examples of the present disclosure have been illustrated, but it has been initially expected to appropriately combine or variously modify configurations of the embodiments and examples.

The embodiments and examples disclosed herein are illustrative and non-restrictive in any respect. The scope of the present invention is defined by the terms of the claims, rather than the embodiments and examples described above, and is intended to include any modifications within the scope and meaning equivalent to the terms of the claims.

### REFERENCE SIGNS LIST

1 tungsten carbide grain; 2 binder phase; 3 cemented carbide; 10 cutting tool; 11 cutting edge.

## Claims

1. A cemented carbide comprising a plurality of tungsten carbide grains and a binder phase, wherein
the cemented carbide includes the tungsten carbide grains and the binder phase in a total of 89% by volume or more,
the cemented carbide includes 1.8% by volume or more and 20% by volume or less of the binder phase,
the binder phase includes 80% by mass or more of cobalt,
the cemented carbide includes an inner region at a distance of 300 µm or more from a surface of the cemented carbide, and
in the binder phase of the inner region, a percentage { S_{(hcp)}/(S_{(hcp)} + S_{(fcc)})} × 100 of an area S_{(hcp)} of cobalt having an hcp structure to a total of the area S_{(hcp)} and an area S_{(fcc)} of cobalt having an fcc structure is 45% or more.

2. The cemented carbide according to claim 1, wherein the percentage {S_{(hcp)}/(S_{(hcp)} + S_{(fcc)})} × 100 is 50% or more and 70% or less.

3. The cemented carbide according to claim 1 or 2, wherein the binder phase further includes at least one first element selected from a group consisting of silicon, phosphorus, germanium, tin, rhenium, ruthenium, osmium, iridium, and platinum.

4. The cemented carbide according to claim 3, wherein in the binder phase, a percentage {M1/(M1 + M2)} × 100 of a mass M1 of the first element to a total M1 + M2 of the mass M1 of the first element and a mass M2 of the cobalt is 1% or more and 6% or less.

5. A cutting tool comprising a cutting edge consisting of the cemented carbide according to any one of claims 1 to 4.
